

Sept. 15, 1931.

W. F. HELMOND

1,823,450

TYPEWRITING MACHINE

Filed Jan. 14, 1929



Inventor:  
William F. Helmond  
by B. G. Stickney  
Attorney

## UNITED STATES PATENT OFFICE

WILLIAM F. HELMOND, OF WEST HARTFORD, CONNECTICUT, ASSIGNOR TO UNDERWOOD ELLIOTT FISHER COMPANY, OF NEW YORK, N. Y., A CORPORATION OF DELAWARE

## TYPEWRITING MACHINE

Application filed January 14, 1929. Serial No. 332,433.

In typewriting machines it is desired to protect against deterioration the key-levers and the bell-cranks by which the key-levers are connected to the type-bars; and another desideratum is that the key-levers and bell-cranks shall be black or dark.

It is also of importance that the touch upon the keys shall be light, and this question of touch involves the working of the joint between the key-lever and the bell-crank, as well as of the joint between the bell-crank and the type-bar. It is therefore desired to protect the entire key-lever and the entire bell-crank, including the joints, and to lighten the operation.

It has been the practice to use a thin metal covering for the key-lever and bell-crank, usually a metal which can be colored black. This result is gained by plating these parts with copper, and then blackening the copper. The copper plating covers the entire lever and the entire bell-crank, including the working studs or bearings which are riveted thereon. This practice has been followed for many years, but it is a feature of the present invention to preserve the aforesaid results as to the key-lever and the bell-crank while effecting a substantial improvement in the action of the keys, with a view to securing smoothness of operation, close fitting of the parts, and other advantages.

The objection to copper for plating the key-levers and bell-cranks, is that copper is a poor bearing material, and it engenders so much friction that it is highly objectionable. Moreover, the copper plating must be of substantial thickness, yet it is difficult or impossible to control this thickness. Hence it is impracticable to produce at low cost, in great quantities, a finely-fitted product.

It has not been practicable to make the plating of copper very thin, because there has to be a substantial coat in order to make it practicable to blacken the copper. Owing to the necessity of making the copper plating so thick, there is an excess of copper so far as the bearing is concerned and various troubles have been encountered.

From time to time the typewriting machines will sweat. The moisture which accu-

mulates upon the type-bars and other parts, and upon the type-bar segments, drops down onto the bell-cranks or links and rusts them, unless they are heavily plated with copper. Rust is a great enemy of the successful manufacture, shipment and sale of typewriting machines.

Other features and advantages will herein-after appear.

In the accompanying drawings,

Figure 1 is a sectional side view of an Underwood type-action with the present invention applied thereto.

Figure 2 is an enlarged sectional view taken on the line 2—2 of Figure 1.

Figure 3 is an enlarged sectional view taken on the line 3—3 of Figure 1.

According to the present invention, in order to improve the touch of the keys 10 for operating type-bars 24 to print against a platen 25, the friction-engendering copper has been eliminated from the bearings of the copper-plated lever 11 and bell-crank 12, and finished, hardened steel studs 13 are riveted to the copper-plated levers 11 and bell-cranks 12, said studs being however cadmium-plated at 14 to protect them from rust, and also to give them lubricous surfaces conducive to much easier operations of the keys.

The thickness of the cadmium coating 14 upon the stud 13 can be predetermined with great accuracy, so that the bearing will fit closely in the slot 15 or 16, in which it works, thus avoiding undue play at the joint, and therefore reducing the depth of key-stroke to a minimum. Since there is considerable working of the stud along the slot at the joint, the use of the lubricous cadmium proves a great advantage. The cadmium has very

great rust-protecting quality, and even if the cadmium coating should in time wear off from the hardened bearing, the cadmium will still remain upon the head 17 or 18 of the stud 13, and the head therefore will not rust, nor will rust appear between the head of the stud and the side of the lever, nor attack the bearing itself. Hence the machine is proof against injury arising from its standing for a long time upon the shelves of the factory,

or in the warehouse, or in boxes during shipment.

5 The cadmium conduces to a light and elastic touch, and effects a substantial improvement over the old method in which the stud was copper-plated as an incident of copper-plating the entire lever, stud and all.

Cadmium forms a hard coating and affords an exceedingly better bearing than copper, 10 and also gives a much better protection against rust. The cadmium remains as a permanent surface on the hardened steel bearing. It forms the best kind of surfacing for the bearing. It does no injury to the bearing itself. There is no necessity of putting on an excess of cadmium, which is a trouble which was constantly met with in coating with copper. The cadmium-coating can be made very thin and of very accurate size.

15 20 The cadmium is put on the bearings by putting the steel bearings in a tumble-barrel which is dipped in a bath of cadmium. The barrel, which is in the form of a tank, is closed up and agitated. Electric contact is made 25 for the purpose of plating the studs with cadmium, while the barrel is revolving. The studs are plated in this way in about ten minutes. The cadmium is self-burnishing, and the studs are found to be brightened. 30 There is therefore no need to rub off or finish the cadmium coatings on the studs, and the cost of manufacturing the completed key-levers and bell-cranks is reduced.

35 The studs may be headed over or riveted at 19 to the key-lever and bell-crank, both of which have been previously plated with copper at 20. The copper-plating extends at 21 within the holes 22 into which the shanks 23 of the studs are inserted before heading 40 over at 19.

45 As against one ten-thousandth of an inch of cadmium plating, the thickness of the copper upon the stud has been practically three or four thousandths. The copper-plating on the levers is subject to a great variation in thickness, while the cadmium-plating is uniform, and the cadmium-plated stud can be made exactly the predetermined diameter and will so remain, and it is unnecessary to 50 give attention to the question of the thickness of the coating or plating, as in practice it is an insignificant matter with cadmium. But copper is subject to great variation in the thickness of the deposits.

55 It will be seen that the rusting of the joints is safeguarded against by the cadmium while preserving the rust-proofing qualities of the copper-coating on the bodies of the key-levers and bell-cranks.

60 Variations may be resorted to within the scope of the invention, and portions of the improvements may be used without others.

Having thus described my invention, I claim:

65 A pivoted lever having an elongated slot

therein and a second lever provided with a pin accurately fitted to move in said slot, said pin having a coating thereon of cadmium approximately one ten-thousandth of an inch thick.

70 WILLIAM F. HELMOND.

75

80

85

90

95

100

105

110

115

120

125

130